

## UNITED STATES PATENT OFFICE.

JOSEPH HAY AMIES, OF PHILADELPHIA, PENNSYLVANIA.

## PAVING COMPOSITION.

No Drawing.

Application filed April 1, 1924. Serial No. 703,541.

*To all whom it may concern:*

Be it known that I, JOSEPH HAY AMIES, a citizen of the United States of America, residing at Philadelphia, in the county of 5 Philadelphia, State of Pennsylvania, have invented a new and useful Paving Composition, of which the following is a specification.

The object of this improvement is to 10 produce the herein specified composition, to be employed particularly, as a surfacing and resurfacing, for streets and highways. It may, however, be used for flooring, roofing and the like.

15 I will now describe the production and application of the composition constituting my wearing surface for highways and the like. I take a given portion of the soil of the grade, and sieve it finely, and then submit it to a blast heater until it attains approximately, two thousand degrees F. of 20 heat. I then take the general soil of the grade in its natural condition and place it within a standard mixing machine. I then 25 wet it with a sufficient amount of boiling hot water to cause it to macerate. I then add from one to two cubic feet of the highly heated soil to every nine to fifteen cubic feet of the common soil of the grade already 30 placed as described within said mixer. I add thereto a sufficient amount of boiling hot water to form a thin macerated soil batter or mortar. The constituency of this mass, at this point, ought to be like that of 35 plaster when prepared to be troweled upon walls or floors. The hot water brought in contact with the highly heated added soil forms a compressive steam thus very rapidly and effectively enabling the full maceration 40 of the soil contents which should now form as stated, a thin mortar. Again, at this point, to every nine to fifteen cubic feet of the soil of the grade thus treated I add from twenty to thirty pounds of pulverized oxide 45 of calcium in a perfectly quick condition, and caused to previously begin to slake. To stimulate and cause the slaking to continue I may add an additional amount of boiling hot water, as by sprinkling. I now 50 add to this macerated and heated soil contents, within the mixer, a due quantity of highly heated bituminous or other pitchy material, and thoroughly mix the same with the contents of the mixer. I have found by 55 this process that the said highly heated bituminous or other pitchy materials are

chemically desirably affected by the slaking of the oxide of calcium. Bituminous or other pitchy materials, after this treatment, will not absorb water or air, and are practically indifferent to the changes of temperature, and will not volatilize or crystallize, but maintain permanently a semi-fluid condition, thus, moreover, by this treatment the soluble salts of bituminous materials 60 become neutralized making water absorption impossible thus preventing oxidation and providing age lasting resistance to wear and tear of traffic. The said composition will give very great solidity of mass when 65 very heavily rolled, tamped and forged and it will accept compression to a perfect extent. This composition, in this condition, it is safe to affirm, will contain less than 70 five percent of voids, and therefore be practically air and water proof. It has been asserted that twenty one percent of voids 75 might be the maximum secured by compression, in bituminous mixtures composed of broken stone and sand fillers, but this degree 80 of inherent stability has never been secured in bituminous compositions having broken stone, sand and gravel contents. Twenty six percentum of voids is the lowest achievement toward securing inherent stability of 85 which we have any record. When bituminous or other pitchy materials are associated with heated mineral or broken stone materials and after the greatest compression has 90 been secured, voids enough will remain to 95 entertain a considerable amount of water which will quickly cause the oxidation and granulation of the said bituminous or pitchy material and thereby result in the premature destruction of the said composition when applied for a street or highway wearing surface. These destructive results I avoid as above affirmed. Moreover, broken stone, sand and gravel owing to the above facts, 100 are capable of considerable vibrations under traffic and will therefore contribute a grinding and friction attrition upon the said bituminous materials stripping them from the mineral aggregates, thereby causing rapid destruction to the highway compositions. In sand, sheet asphalt, the voids are never 105 reduced to less than thirty-two percent, consequently this composition may entertain large quantities of water.

The said bituminous or other pitchy materials should preferably have a penetration of about 60 or 65, so that when they 110

come to the temperature of the air they will be tough enough, when duly condensed by compression as by rolling and tamping and forging, to resist, without indentation the 5 heaviest truck traffic tonnage. This surfacing and resurfacing composition should be placed upon a sub-foundation compressed, as described, to the fullest degree of solidity, practicable. The said sub-foundation should 10 be placed upon a fine grade, also constructed so as to secure the greatest practical degree of compression.

Preferably, I employ a very highly heated bituminous or other pitchy material, 15 because, in the first place, it is much cheaper, and in the second place, the street or highway surfacing or resurfacing, will submit to traffic, as soon as it comes to the temperature of the air, which is, usually, 20 in about four to six hours. But these desirable results cannot always be determining factors, because conditions and conveniences may dictate terms in favor of the employment of a cold liquid, bituminous or other 25 pitchy material, such as naphtha cutback or any other form of emulsified bituminous or other pitchy material. The difference in cost between the heated bituminous material and the cold liquid state thereto 30 may not be as great as it seems to be, at first sight, because, notwithstanding, the cold liquid form of bituminous material may be one-third higher than the hot liquid used, yet the preparation and extra costs 35 of labor and equipment employed to secure the heated article, may considerably lessen this difference in costs. Then, again, in many cases, convenience may outweigh all. But after all is said, the hot application is 40 preferable, because it will be considerably cheaper, and become, as said, ready for service as soon as it arrives at the temperature of the air. And furthermore, and more important than all other considerations, it 45 will greatly outlast the wearing resistance of any form of cold application of emulsified asphaltum. Nevertheless, convenience may make, in some cases, the cold application of emulsified asphaltum, desirable, but 50 this can only occur in isolated instances. It is to be observed that bituminous material always inter-absorbs the soil, it does not coat units thereof but interfuses them, and therefore a complete inter-amalgamation 55 takes place. Owing to this, very intense solidification is attained, and the evaporation of the volatile and essential

oils, is prevented, therefore, the composition made with cold liquid asphaltum material, in most cases, becomes impractical, because, it might take months before the surfacing and resurfacing of the streets or highways would become tough enough to entertain traffic, notwithstanding the fact that the cold liquid asphaltum would come 60 in contact with the heated soil.

The highway wearing surface should be homogeneous with the density and colloidal disposition of a properly blown vehicle or rubber cast tire. And again the sub-foundation should be homogeneous with the wearing surface. And furthermore, the fine grade should be harmonious with, although less resistance than, the surfacing and sub-foundation, but altogether should 70 homogeneously relate, as above described, with properly provided vehicle tires. When this is secured the vibrations of shock and attrition will be infinitely divided and subdivided and dissipated and the entire 75 traffic will be accepted by a sympathetic cushion like enduring superstructure.

It will be seen that I have described a highway superstructure, giving the foregoing desirable qualities at a very low cost 80 possessing complete scientific adaptation resulting in the finest qualities and greatest endurance for highway traffic.

Having fully described the production of a bituminous composition to serve as a 85 wearing surfacing and resurfacing superimposed upon, and related to, already devised and placed perfect fine grade and sub-foundation;

What I claim is:

1. The process of making a bituminous paving composition consisting of subjecting one-tenth portion of the natural soil of the grade to a temperature of about 2000 degrees F., in a blast heater, placing the 100 balance of the natural grade soil in a mixing machine and macerating with boiling hot water then adding the foregoing heated soil to the contents of the mixer, then adding to each 9 cubic feet of this highly heated mass 20 to 30 pounds of finely granulated quick lime, and finally adding a quantity 105 of bituminous material in a highly heated state.

2. The paving composition produced by 110 the process of claim 1.

In testimony whereof I have hereunto signed my name.

JOSEPH HAY AMIES.